

Aug. 7, 1945.

D. S. PHELPS

2,381,514

SETTLING OF PHOSPHATE ORE MATERIALS

Filed Oct. 13, 1942

4 Sheets-Sheet 1

Fig. 1

Fig. 2

SEDIMENTATION BY  
CAUSTIC SODA-SODIUM SILICATE



SEDIMENTATION BY  
CAUSTIC SODA-SODIUM SILICATE



Fig. 3



INVENTOR:  
Donald S. Phelps  
BY

John C. Kerr  
His ATTORNEY

Aug. 7, 1945.

D. S. PHELPS

2,381,514

SETTLING OF PHOSPHATE ORE MATERIALS

Filed Oct. 13, 1942

4 Sheets-Sheet 2

*Fig. 4*



*Fig. 5*



*Fig. 6*



INVENTOR:

Donald S. Phelps

BY

John C. Kerr  
His ATTORNEY

Aug. 7, 1945.

D. S. PHELPS

2,381,514

SETTLING OF PHOSPHATE ORE MATERIALS

Filed Oct. 13, 1942

4 Sheets-Sheet 3



INVENTOR:

Donald S. Phelps

BY

John C. Kerr

His ATTORNEY

Aug. 7, 1945.

D. S. PHELPS

2,381,514

SETTLING OF PHOSPHATE ORE MATERIALS

Filed Oct. 13, 1942

4 Sheets-Sheet 4



Fig. 10



Fig. 11



Fig. 12

INVENTOR:

Donald S. Phelps  
BY

John C. Kerr  
His ATTORNEY

## UNITED STATES PATENT OFFICE

2,381,514

## SETTLING OF PHOSPHATE ORE MATERIALS

Donald S. Phelps, Harvard, Mass., assignor to The American Agricultural Chemical Company, New York, N. Y., a corporation of Delaware

Application October 13, 1942, Serial No. 461,886

7 Claims. (Cl. 209—5)

This application is a continuation-in-part of my copending applications Serial No. 359,642, filed October 4, 1940 (Case 1); Serial No. 393,888, filed May 17, 1941 (Case 2); Serial No. 393,889, filed May 17, 1941 (Case 3); Serial No. 433,162, filed March 3, 1942 (Case 5); and Serial No. 439,028, filed April 15, 1942 (Case 6).

The present invention relates to a fundamental discovery which I have made in the art of phosphate mining and recovery, namely, that a certain class of chemical reagents, which, for convenience, I have designated as "phosphate ore sedimentation-acceleration reagents," or "settling-acceleration" reagents, as I sometimes call them, and which are hereafter described, defined and illustrated, have the remarkable property of producing a greatly accelerated rate of sedimentation or settling of aqueous suspensions, pulps or slurries of phosphate ores, when the reagents are added thereto in relatively small and economical quantities, and, generally, but not always necessarily, in an alkaline state, or with, or in the presence of, an alkaline reagent.

The invention relates specifically to the treatment of phosphate ores; and, in particular, to a process for treatment and recovery of such ores wherein an aqueous suspension, pulp or slurry of the ore, or part of it, more especially the finer particles thereof (many of which are too fine to settle rapidly even in still water), is subjected to "accelerated sedimentation" by treatment with one or more of my novel "sedimentation-acceleration" reagents of the class referred to, and the thus-settled material is then recovered or collected, and then subjected to various separation treatments for separation and concentration of valuable phosphate materials, including those which would otherwise go to waste, or which could not be recovered for a long time.

Objects of the invention include attainment of the results just stated.

In the usual hydraulic process of mining phosphate ore, more especially Florida pebble phosphate, which does not require crushing or grinding, the overburden of earth is first removed and the exposed banks of phosphate ore (containing the phosphate mineral or "phosphate rock") are then hydraulically mined, by means of streams of water under high pressure. The resulting slurry is then pumped to a phosphate washer or recovery plant, often known generically in the industry, as a "washer," and sometimes so referred to in the following description. This "washer" usually includes a washing, screening and hydraulic-separation or classification installation,

followed by tabling, flotation, sometimes electrostatic separation, and perhaps other concentration steps carried out in suitable apparatus.

The feed from the hydraulic mining operation to the "washer" may include pieces of phosphate rock from about two inches or more in size down to material that will pass through a 325 mesh screen—that is, material which may be smaller than 0.0017 inch in diameter, and much of it is so small that it will settle only very slowly, or not at all, from an aqueous suspension. The feed to the "washer" also usually contains a certain amount of sand or quartz, clay, and perhaps other impurities and waste material. At the washer, the feed is ordinarily agitated, washed, screened, hydraulically classified, and the smaller sizes of phosphate mineral, say less than about 20 mesh, are then, in many plants, concentrated from the impurities and waste by flotation, sometimes preceded by tabling and other separation processes.

Another method of phosphate mining, sometimes employed on domestic ores, including Florida deposits, is the so-called "dry-mining" process, according to which the phosphate-bearing ore is dug out in dry condition, as by a scoop or shovel, and may be thereafter soaked in water or otherwise disintegrated, after which the material may be subjected to hydraulic classification, flotation and other treatment.

Altogether, therefore, several different methods of separation are often used; and in hydraulic mining these may occur in different parts of the complete "washer" or phosphate washing and concentration plant. The various steps, in both forms of mining, may include hydraulic classification, screening, tabling, as by shaking tables, with or without oiling, flotation, settling and sometimes electrostatic separation—the several different methods being used sometimes separately in different parts of the plant, and sometimes together, either in succession or in combination.

During all these operations, the finer sizes of phosphate mineral, usually less than approximately 65 mesh, and sometimes considerably coarser, and almost always the material finer than 100 mesh, tend to remain suspended in the water, together also with the finer particles of silica, sand, clay or other impurities present. This is especially so in the overflow product from the settling tanks, and particularly when the flow of water through such tanks is relatively rapid. Because of economic factors, the tanks are necessarily relatively small compared to the total volume of water. Therefore, there is usually a rapid

flow through them, giving a relatively short time for settling. In some installations this time may be, for example, between a minimum of about 5 seconds and a maximum of about 30 seconds, as shown by actual measurement; and in other installations it may be between about one and two minutes. Because of this rapid flow, and short time in the settling zones, much unsettled fine material ordinarily passes out to the "debris dump" or "settling pond" where, over a period of months or years, it may, to some extent at least, go through a natural, but very slow, process of settling and "de-sliming." After standing for months, or sometimes years, in the debris dump or settling pond, some of the material may be pumped back out of the pond and returned to the "washer," or some part of the plant, for re-treatment and concentration.

Even when such re-treatment of the debris is ultimately possible, the delays are great and the phosphate losses are high. Also, repumping the material may tend to put the fine particles back in suspension. In addition, the expense of pumping the washer or settling-tank overflow product first to the debris dumps or settling ponds, and later back for re-treatment, is considerable, because of the power and labor required, and there is a long delay while natural settling takes place.

For a period of many years this problem has been a fundamental, and perhaps the principal, one among those engaging the attention of phosphate producers; and because the field is highly competitive and costs are extremely important, long and repeated efforts, by many leading engineers in the field, have been made, to find some practical solution for the problem of improving the recovery of this unsettled fine phosphate material, and to overcome the necessity for re-pumping and re-treating the debris.

My present discovery includes the fact that by a relatively simple and economical treatment with one or more of the "phosphate ore sedimentation-acceleration" reagents previously referred to, and which are hereafter described and illustrated in detail—which treatment is applicable, if desired, either to the initial feed from the mine to the entire "washer" (i. e., to the phosphate ore treating plant as a whole), or to other appropriate stages of the process, but which I have found preferable when applied directly in the settling tanks, or in the feed thereto—it is possible to treat the suspended material, including the phosphate mineral and impurities alike, in such a way that its settling is greatly accelerated, and the recovery of both the settled phosphate mineral and the impurities is greatly improved; after which the thus-settled material may be concentrated and the desired phosphate recovered.

My novel treatment has been found to increase the total recovery of solids in the settling tanks, especially when the reagent is added at that point in the process, and the treatment may be carried out to such an extent as to obviate the necessity of re-pumping and re-treating the debris from the debris dumps or settling ponds. It may thus result in very substantial savings, both in the recovery of phosphate (i. e. phosphate mineral) and in the cost of the process, including a saving of power in re-pumping the debris, of labor costs, and in preventing delay.

Figures 1 and 12 hereof, more particularly described hereafter, are illustrative examples of results obtained by various treatments according to my invention. By way of an illustrative ex-

ample of the arrangement of what may be regarded as a typical phosphate washer in the case of an hydraulic mining operation for unground Florida pebble phosphate, upon which my treatment has been found especially effective, the feed, as pumped from the mine, passes first through a hammer mill (i. e., a beater type of mill), which disintegrates the mud balls, thence by flumes to a sump. The pulp is then pumped to a set of 10 dewatering screens and the water, containing all of the solids finer than approximately fourteen mesh, then goes to the sedimentation tanks and thence to the concentration plant. The oversize or plus 14 mesh goes to several sets of screens and scrubbers which wash and separate the finer particles stuck to the oversize particles, so that much of what was originally oversize eventually goes back to the sump and, if it has been further disintegrated in the meantime, has a second opportunity of becoming part of the undersize of the head screens. In this way the ore masses of phosphate mineral, clay, sand, and all other impurities become well disintegrated and particularly all the fine particles eventually reach the settling or sedimentation tanks.

The minus fourteen mesh material which eventually reaches the sedimentation tanks is there offered a brief opportunity to settle and that portion which does settle forms the feed to the concentration plant proper. The overflow or effluent of the sedimentation tanks, containing all the particles which do not settle while in the sedimentation tanks, including phosphate rock, clay, silica and other impurities, goes from the settling tanks to the settling area or ponds, which is a very large ground area dammed off for the express purpose of settling the solids from the water. This area may be very extensive, for example, a matter of one mile square or even more.

The flow through the "settling tanks" is necessarily relatively rapid, as already indicated, since it is impractical, economically, to have the tanks large enough, and to allow the liquid to remain in them for a sufficient time, to make a full natural separation or settlement of the solids. The latter usually occurs only over a period of months or years, in the settling ponds; while the time allowed for settling in the "sedimentation tanks" may be a matter of minutes, or even, perhaps, of seconds in some cases. For example, in one illustrative installation, the time of flow across the surface was found to be between a maximum of about 30 seconds down to a minimum of about 5 seconds; while even in a very large settling tank of modern design, the time available for settling may be only of the order of about one to two minutes, or less, with an average of about 30 seconds under certain conditions. Thus, in the absence of treatment to produce accelerated settling, the overflow product from the settling tanks usually consists of a muddy liquid in the form of a pulp, suspension or slurry, which may still contain a very substantial quantity of valuable phosphate mineral, mixed with silica and other impurities, but which heretofore, it has been impossible to settle and concentrate economically, or in any practical manner, either in the settling tanks or in any other part of the plant. Not only was it impossible to separate the unsettled solids, effiently, for any sort of subsequent treatment, but particularly by reason of the necessary hydraulic mining or washing or soaking operations, the settling tank overflow, and indeed the feed to the settling tanks as well, have been too dilute for efficient wet concentration, as by flotation, ta-

bling, and so forth. A sample of this pulp (overflow product from the settling tanks), allowed to stand quietly in a tall graduate, is usually found to settle very slowly, and sometimes not perceptibly within a short period of observation.

A feature of the present invention resides in the discovery that by the addition of a relatively small and economical quantity of one or more of my newly discovered "phosphate ore sedimentation acceleration" ("settling acceleration") reagents, either directly to the settling tanks, or to the feed thereto (although it may be done at other suitable stages of the process), the settling of this finer material, including phosphate mineral and impurities alike, can be very greatly accelerated, so that the subsequent concentration and over-all recovery, after settling, is much improved, even when the time in the settling tanks is only of the order of those stated above. Thus the importance of a high initial settling rate will be seen, so that the amount of solids settled out will be high during the initial period of settling.

Addition of the reagent or reagents may be in the presence of, or accompanied by, an alkaline reagent such as caustic soda, or may be made to the pulp or suspension when in an alkaline condition.

My novel "phosphate ore sedimentation-acceleration reagents" are characterized and may be distinguished by being water miscible (which term, as used herein, includes both soluble and suspensible), and by having a common action, of the character already stated, upon phosphate ore pulps, aqueous suspensions or slurries. That is to say, when the reagent is applied, in relatively small, and economical, quantity, to an aqueous suspension of phosphate ore which is composed of, or includes, particles of both phosphate mineral and intermixed impurities, which are either too fine to settle rapidly in flowing, or even in still water, or will not settle at all under such circumstances, the reagent produces a markedly accelerated settling—in some cases a settling where none would otherwise occur, or at least, be observable, within any reasonable time—and generally of the phosphate particles and impurities alike. This may produce a very substantial amount of settling within the first minute or two minutes of settling time elapsing after treatment, even where no such settling would otherwise occur; and in many instances there may be a substantial initial settling during the first 30 seconds available for settling, elapsing after treatment with the reagent. Even when the reagent is added to the pulp well in advance of the settling tanks, its effect persists so that rapid settling occurs as soon as opportunity is presented. In other cases, it is to be observed that my reagents, when applied in the amounts and concentrations indicated by the examples given below, have the effect of more than doubling the volume of settled material, as compared with material not so treated with the reagents, at all times throughout a short initial settling period such as already indicated—and even in some cases throughout about the first three minutes of settling time, as indicated by the examples to be given; the increase of the rate of settling being of the intermixed fine particles of both phosphate and impurities, as compared with their untreated settling rate.

In general, the action of my novel reagents is not one of separation or selection, but is a more rapid settling of all the materials substantially alike, including both phosphate and impurities, as

is shown by analysis of the material before settling and of the settled product collected after treatment. In general, these are found to have much the same percentage composition, indicating that the accelerated settling treatment does not produce a separation of the phosphate mineral from the silica and other impurities, but causes a more rapid settling of both alike.

10 This common action upon phosphate ore suspensions is a striking common characteristic of my novel class of materials, and is an important feature by which they can be determined and recognized.

15 Another means of identification of my novel class of reagents is that all of them, so far as I know, are, and many of them are known to be, deflocculating or dispersing agents for various materials. Many of them have been suggested or used for various separating, deflocculating, dispersion or flotation applications, as regards a 20 variety of materials and ores, some of them for phosphate materials; but the mere fact that the material is so known as a deflocculating or dispersing agent, for another ore or even for phosphate, is not, so far as I am at present aware, a sufficient criterion to determine or predict with certainty, whether it falls within the present 25 class of phosphate ore settling-acceleration reagents. That is to say, the possession of deflocculating or dispersing properties is, as at present 30 advised, a necessary but not a self-sufficient condition for successful use in my process.

35 According to my best present information, certain deflocculating or dispersing agents, previously known or suggested for that purpose in connection with various ores, do not possess, to any substantial degree, the property of producing accelerated settling of phosphate ores; and hence are not within the class of materials which I have 40 discovered, and claim herein. Examples of such reagents are: agar agar, gum acacia and black-strap molasses, all of which have long been known as deflocculating or dispersing agents for various ores, but which do not possess, to any substantial degree, the property of producing accelerated settling of phosphate ores.

45 A further test, and one which, as at present advised, I believe to be a sufficient as well as a necessary condition, for determining whether a given deflocculating agent does or does not fall within my novel class of reagents, is that the material must be one which is water miscible (which term, as used herein, includes both soluble and suspensible) and which, when so mixed, whether such mixture be by suspension or solution, is 50 capable of dispersing, in water, one or more colloidal constituents of phosphate ore, in the presence of insoluble calcium phosphate. So far as at present advised, that test is a definite means of identification of my novel class of compounds.

55 Preferably, too, but not necessarily, the reagent is either itself alkaline in reaction, or possesses the foregoing property when in an alkaline solution, suspension or medium, as in the presence of an alkaline reagent.

60 So far as I am at present aware, their common action upon phosphate ore suspensions, as already described, and the other criteria given above, are the best available and most definite means of identifying and defining my novel class of compounds as generically defined and claimed herein; but the description and identification is also promoted by illustration. Thus, as illustrative, but not exclusive, examples of my novel 65 class of materials, the following are given, and

these include the best materials now known to me for the purpose. They are, in general, either themselves alkalis or are preferably employed to advantage in an alkaline state or condition, or in the presence of, or simultaneously with, an alkaline reagent, such as, for example, caustic soda, either added separately or included with the reagent. The illustrative examples of suitable reagents follow:

(1) Sodium silicate ( $Na_2SiO_3$ ), and preferably having a composition of approximately



and preferably added in an alkaline state, or together with caustic soda, and suitably in the proportions of sodium silicate and caustic soda hereafter further illustrated.

(2) Molecularly dehydrated alkali phosphates, including, specifically, tetra-sodium pyrophosphate ( $Na_4P_2O_7$ ), dissolved or in solid state, and sodium metaphosphate ( $NaPO_3$ ).

(3) Lignin sulfate, lignin sulfonate and lignin sulfite products, including wood pulp waste liquors; specifically the trade-marked products known as Daxad No. 11 and Daxad No. 23, sold by Dewey & Almy Chemical Company of Cambridge, Massachusetts; Black Liquor; Goulac and Glutrin, trade-marked products sold by Robeson Process Co., of New York.

Of the foregoing materials, my best present information is that Daxad No. 11 and Daxad No. 23 are both lignin sulfonate products; Black Liquor, as sold by the West Virginia Pulp and Paper Co., of New York, is a by-product of the paper industry, generally made from pine wood and containing a lignin sulfate. Goulac is a lignin sulfite product derived from wood pulp waste liquor as sold by the Robeson Process Co., of New York. This is sold in the form of a solid. Glutrin is a lignin sulfite derived from wood pulp waste liquor and also sold by the Robeson Process Co., of New York. This is sold in the form of a liquid of 50% strength.

(4) Tri-sodium phosphate, or any sodium orthophosphate in the presence of a sufficient quantity of an alkaline reagent (e. g., caustic soda) to effect conversion to tri-sodium phosphate.

(5) In the case of certain phosphate ores, apparently those taken from particular localities, (e. g. ore mined in the neighborhood of Hopewell, Florida (I have also found that caustic soda when used alone, for example in the proportions of about 0.5 pound or 1.0 pound of caustic soda per ton of feed, produces advantageous results, and may, in some cases, produce results comparable with those obtained with the other reagents named above. This is not true, however, of all ores; and I have not ascertained the reason for the effectiveness of caustic soda alone in certain cases. It appears, however, to be due to some difference in the composition of the ore, the exact nature of which I am at present unable to explain.

The effect upon various samples of commercial grades of phosphate or pulps or suspensions, of accelerated settling treatment with certain of the foregoing sedimentation-acceleration reagents, is illustrated in the accompanying drawings, it being understood that different results may be obtained upon different samples of ore from the same locality, or upon ore from different localities, or upon samples of different ages, or which have stood for varying periods. The foregoing and many other factors may affect the result;

hence the accompanying curves are illustrative only:

In making all these curves a sample of the pulp was placed in a 1000 cc. graduate and the measured amount of reagent and caustic added. The mixture was agitated and then allowed to stand. On standing quietly small particles of phosphate and impurities settle, although the supernatant water remains turbid. The body of solids settled in the liquid at and near the bottom of the graduate can be readily seen, and generally exhibits a reasonably definite line (actually, surface) of demarcation between it and the turbid supernatant liquid. The increasing volume of settled solid in the bottom of the graduate is then read (in cc.) on the scale of the graduate from time to time (without removing or otherwise disturbing the supernatant liquid) and these values are plotted against the time (in minutes) to give the settling curves shown in the figures. Unless otherwise stated, reference anywhere herein or in the claims to the volume of solids settled or recovered, means the volume measured wet, as just described.

The pulps employed for these tests were derived from commercial phosphate washer or treating plants, and are believed to be representative of a number of types of pulp or suspended ore that may be found in such plants; for variety, some pulp (as for the Fig. 1 test) was taken from the overflow or "waste" of previous sedimentation tanks (which did not embody my process) and some (for the Fig. 7 and 8 tests) was derived by re-pulsing, in a manner that is commercially required for removal and handling, the material from phosphate debris banks produced by the large or "waste" settling ponds mentioned hereinabove.

Figure 1 is an illustrative accelerated-sedimentation curve illustrating the effect of treatment of a one-liter sample of an aqueous phosphate suspension taken from the overflow product from a settling tank, with a settling acceleration reagent consisting of 5 cc. of a 5% solution of caustic soda and 30 cc. of a 5% solution of sodium silicate ( $Na_2SiO_3$ ), equivalent to 1.4 pounds of caustic soda and 8.8 pounds of sodium silicate per ton of solids in the sample pulp (suspension) under test.

In the curve marked "treated," the effect of this treatment is shown, as contrasted with the effect produced by natural settling when no reagent was added to a similar sample of the same suspension, marked "untreated."

Figure 2 is a similar illustrative curve showing the effect of treatment with caustic soda and sodium silicate. In this particular sample the total solids amount to 200 grams in a volume of feed pulp amounting to 1000 cc. The reagents were employed in the proportion of 1.0 pound of caustic soda and 2.0 pounds of sodium silicate 40° Bé. per ton of solids in the feed pulp.

Figure 3 is also illustrative of the results produced upon a different sample by treatment with caustic-soda and sodium silicate. In this instance the treatment was with 2.0 pounds of caustic soda and 4.0 pounds of sodium silicate 40° Bé. per ton of solids in the pulp treated. In this sample the total solids amounted to 252 grams in a volume of pulp amounting to 1000 cc.

Although no illustrative curves are given showing the results of treatment with caustic soda alone, for the reason that it appears to be effective only in the case of particular ores, or ore taken from particular localities, I have never-

theless obtained good results in certain instances, upon ore from the Hopewell (Florida) district. Upon certain samples of Hopewell ore I obtained results roughly comparable with those illustrated in Figure 2, by treatment of a sample comprising 200 grams of solids in a 1000 cc. volume of pulp with a caustic soda solution equivalent to 1.0 pound of caustic soda per ton of solids in the pulp feed; and on another sample of such ore, containing 210 grams of solid in a 1000 cc. volume of pulp, I obtained good results by treatment with caustic soda equivalent to 0.5 pound per ton of solids in the pulp feed. These results, however, were only obtained upon an unusual sample exhibiting a condition of partial deflocculation after treatment with caustic soda.

In Figure 4 there are shown illustrative examples of curves of sedimentation, for untreated phosphate-bearing material and for the same material treated with an aqueous solution of 5% tetra-sodium pyrophosphate ( $Na_4P_2O_7$ ) in the proportion of 75 cc. of the solution to 500 grams of solids. The pulp had a specific gravity of 1.308 with a quantity of solids in the pulp amounting to 38.3% by weight. In this particular test the volume of the settled solids amounted to about 326 cc. per liter after 16 minutes settling time, and the settling-acceleration reagent was employed in the proportion of 15.0 pounds of reagent per ton of solids in the pulp being treated.

From these illustrative curves it may be noted that, on the particular sample of phosphate material tested, there was a very rapid settling during the first two or three minutes of settling time, when the settling-acceleration reagent was first added. This is of importance in carrying out a commercial process, because it is ordinarily possible to retain the suspension in the settling tanks, for example, for only a very brief period of settling; often less, even, than three minutes, and very generally less than 8 to 10 minutes; and in some cases even less than 30 seconds or one minute, since the flow through the tanks is of necessity very rapid.

Figure 5 shows similar illustrative sedimentation curves illustrating the results obtained by use of dry solid tetra-sodium pyrophosphate. In this case the data were:

Specific gravity of pulp ..... 1.308  
Percent solids in the pulp ..... 38.3  
Weight of solids ..... grams 500

The reagent used was 5 grams of dry solid tetra-sodium pyrophosphate per liter of pulp, equivalent to 20 pounds of the reagent per ton of solids in the pulp.

In the case of this particular sample under treatment, it is to be noted that while the untreated material was not observed to settle at all, within the period of time covered by the observations, there was a very rapid settling of the treated material within the first three minutes. In addition to the advantages pointed out in connection with Figure 4 above, there was thus, in this case, a very material increase in the total volume of settled material recovered. This is of importance in cases where a maximum recovery is necessary. Although that can seldom be obtained economically in plant practice under present economic conditions, it may be of extreme importance wherever supplies or natural resources are limited, e. g., under war conditions.

Figure 6 comprises similar illustrative settling curves obtained by the use of dry sodium meta-

phosphate ( $NaPO_3$ ). In this particular example the conditions were as follows:

Specific gravity of pulp ..... 1.228  
Percent solids in the pulp ..... 30.2  
Weight of solids ..... grams 371

The reagent used was 0.5 gram of dry, solid sodium metaphosphate per liter of pulp, equivalent to approximately 2.70 pounds of reagent per ton of solids in the pulp. In this case, no alkaline reagent was used, and the sodium metaphosphate employed was not alkaline in reaction when dissolved in water.

It will be seen that, on the particular sample tested, the reagent had the advantage of producing a very rapid settling within the first minute; and also that it produced a substantial recovery of the solid material when treated, although the untreated pulp, in this instance, showed no observable settling within the period of observation.

In Figure 7 there are shown illustrative examples of curves of sedimentation, for the normal (i. e., untreated) material in the case of a pulp having a specific gravity of 1.220, with a percent 25 of solids in the pulp amounting to 29.3%; the weight of the dry solids amounting to 357 grams per liter; and for the same material when treated with a settling-acceleration reagent comprising Daxad No. 11, in the proportion of approximately 30 seven pounds of reagent per ton of solids in the pulp being treated, and with caustic soda solution in the proportion of about 2.80 pounds of dry 35 caustic soda per ton of solids in the pulp. The pulp used for this test (Fig. 7) consisted of a suspension of phosphate "debris," i. e. a mixture 40 of phosphate mineral and impurities, which was taken from the phosphate "debris dumps" mentioned hereinabove; the pulp having characteristics representative of the result of operations such as are necessary for repulping and handling such debris.

In this case, also, it is to be noted that there was a marked increase in the volume of sediment obtained in the first one or two minutes of settling 45 time when the settling acceleration reagent was used, and that there was a material increase in the total volume of sediment recovered.

Figure 8 shows similar illustrative curves, illustrating the results obtained by use of Daxad No. 50 23. In this case a "debris" pulp like that used for Fig. 7 was employed, and the data were:

Specific gravity of pulp ..... 1.220  
Percent solids in pulp ..... 29.3  
Weight of solids ..... grams 357  
Pounds of dry caustic soda per ton of solids 2.80  
Pounds of Daxad No. 23 per ton of solids ..... 5.60

Figure 9 comprises similar illustrative curves obtained by the use of black liquor. In this example, the conditions were as follows:

Specific gravity of pulp ..... 1.220  
Percent solids in pulp ..... 29.3  
Weight of solids ..... grams 357  
Pounds of dry caustic soda per ton of solids 2.80  
Pounds of black liquor per ton of solids ..... 8.14

Figure 10 shows similar comparative settling curves for treated and untreated materials in the case of treatment with Goulac and caustic soda. 70 1000 cc. of the pulp contained 371 grams of solids and were treated with 2.0 grams of Goulac and 0.6 gram of caustic soda.

Figure 11 is a similar set of comparative curves in the case of treatment with Glutrin and caustic soda; 75 1000 cc. of the pulp contained 371 grams of

solids and were treated with 25 cc. of liquid Glutrin, of a concentration of 10% by volume, and 0.5 gram of caustic soda.

In Figure 12 there are shown illustrative examples of curves of sedimentation, for the normal (i. e., untreated) material and for the treated material in the case of treatment with tri-sodium phosphate in the presence of caustic soda. The pulp under test had a specific gravity of 1.238 with a percent of solids in the pulp amounting to 31.2% by weight. In this particular case the weight of the solids amounts to 376 grams per liter and the tri-sodium phosphate was employed in the proportion of about 26.60 pounds of tri-sodium phosphate ( $Na_3PO_4$ ) per ton solids in the pulp, and with caustic soda solution in the proportion of 2.66 pounds of dry caustic soda per ton of solids in the pulp.

Tests have revealed that in operations of the sort exemplified by all of the foregoing examples, the composition of the settled material (after drying) is approximately 35% BPL (bone phosphate of lime), and that in general, the settled and dried material will all pass a 10 mesh screen, while about 95% of it is retained on a 325 mesh screen.

For convenience of reference and comparison, I have summarized the data of the tests in the form of a composite table.

change in the composition of the settled material, as between phosphate and impurities. The material thus recovered by settling may be thereafter subjected to hydraulic classification, tabling, flotation, or any other appropriate process for concentration and recovery of the desired phosphate material.

From an examination of the foregoing illustrative curves it will be observed (for example see Figure 1) that it is a property of many of my novel reagents that when they are applied to a suspension of finely divided particles of both phosphate and impurities, even when the particles are too fine to settle rapidly from such an aqueous suspension, the appropriate amounts and concentrations of the settling acceleration reagents, as illustrated above, are sufficient in amount and concentration to more than double the volume of settled material, as compared with material not so treated, at all times throughout an initial short period—for example, the first three minutes—of settling time (compare Figure 1), and sometimes throughout even longer periods as shown by the other examples, such increase of the rate of settling being of the intermixed fine particles of both phosphate mineral and impurities, as compared with their untreated settling rate.

Tests with settling-acceleration reagents, on Florida phosphate ore pulps

| Test | Reagents                        | Reagent, lbs./ton of solids in feed pulp | Caustic, lbs./ton of solids in feed pulp | Percent solids in feed pulp <sup>1</sup> | Specific gravity of feed pulp | Grams solids in feed pulp <sup>2</sup> | Volume of settled product |               |              |               |              |               | Ratio in percent <sup>3</sup> |  |
|------|---------------------------------|------------------------------------------|------------------------------------------|------------------------------------------|-------------------------------|----------------------------------------|---------------------------|---------------|--------------|---------------|--------------|---------------|-------------------------------|--|
|      |                                 |                                          |                                          |                                          |                               |                                        | After 1 min.              |               | After 2 min. |               | After 3 min. |               |                               |  |
|      |                                 |                                          |                                          |                                          |                               |                                        | Natural, cc.              | Acceler., cc. | Natural, cc. | Acceler., cc. | Natural, cc. | Acceler., cc. |                               |  |
| 1.   | Sodium silicate                 | 8.8                                      | 1.4                                      | 35.7                                     | (1.275)                       | (450)                                  | 13                        | 90            | 30           | 100           | 40           | 105           | 65.7                          |  |
| 2.   | Sodium silicate (40° Ré. soln.) | 2.0                                      | 1.0                                      | 20.0                                     | (1.110)                       | 200                                    | None                      | 90            | None         | 110           | None         | 116           | 83.0                          |  |
| 3.   | do                              | 4.0                                      | 2.0                                      | 25.2                                     | (1.145)                       | 252                                    | 45                        | 146           | 77           | 158           | 100          | 163           | 89.6                          |  |
| 4.   | Tetra sodium pyrophosphate      | 15.0                                     | 0.0                                      | 38.3                                     | 1.308                         | 500                                    | None                      | 250           | None         | 300           | None         | 320           | 94.2                          |  |
| 5.   | do                              | 20.0                                     | 0.0                                      | 38.3                                     | 1.308                         | 500                                    | None                      | 250           | None         | 300           | None         | 340           | 89.6                          |  |
| 6.   | Sodium metaphosphate            | 2.7                                      | 0.0                                      | 30.2                                     | 1.228                         | 371                                    | None                      | 200           | None         | 210           | None         | 210           | 91.6                          |  |
| 7.   | Daxad #11                       | 7.0                                      | 2.8                                      | 29.3                                     | 1.220                         | 357                                    | 40                        | 212           | 170          | 233           | 210          | 240           | 89.0                          |  |
| 8.   | Daxad #23                       | 5.6                                      | 2.8                                      | 29.3                                     | 1.220                         | 357                                    | 90                        | 230           | 170          | 230           | 210          | 250           | 100                           |  |
| 9.   | Black liquor                    | 8.14                                     | 2.8                                      | 29.3                                     | 1.220                         | 357                                    | 80                        | 210           | 170          | 246           | 210          | 250           | 100                           |  |
| 10.  | Goulae                          | 10.8                                     | 3.24                                     | 30.2                                     | 1.228                         | 371                                    | None                      | 175           | None         | 195           | None         | 200           | 100                           |  |
| 11.  | Glutrin (50% soln.)             | 27.0                                     | 2.7                                      | 30.2                                     | 1.228                         | 371                                    | None                      | 165           | None         | 190           | None         | 190           | 100                           |  |
| 12.  | Trisodium phosphate             | 26.6                                     | 2.65                                     | 31.2                                     | 1.238                         | (380)                                  | 45                        | 170           | 85           | 200           | 142          | 220           | 88.0                          |  |

<sup>1</sup> By weight.

<sup>2</sup> In 1000 cc. of feed pulp.

<sup>3</sup> Volume of solids after 1 min./volume of solids after 15 min. (both measured on the treated pulp).

Parentheses ( ) indicate calculated values.

From the foregoing illustrative sedimentation curves it will be observed that my process has at least two outstanding advantages. It greatly accelerates the settling by treatment with the reagents in question, thus permitting a recovery of material which would otherwise be lost because the pulp could not economically be left in the settling tank long enough to catch it; and it permits the recovery by sedimentation of fine material, by treatment with my newly-discovered acceleration reagents, even under conditions where no material at all would be recovered by sedimentation, within the observed periods, as shown on the accompanying curves.

It is to be understood, also, that my invention is not primarily directed to any selective separation or concentration of phosphate or phosphate ingredients per se; on the contrary, it is a method of producing an accelerated settling of fine particles of phosphate materials together with silica and other impurities. It permits the rapid settling and recovery of solids in the pulp which would otherwise be lost, but without substantial

In other instances, with certain of the most rapid of my reagents (compare Figure 6, for example), there is produced a very rapid settling within an initial short period of sedimentation—e. g., the first minute, in the case of the treated material, even though no observable settling of the untreated material occurred at any time within the period of observation, in that instance amounting to sixteen minutes. That is to say, my novel reagents may produce settling of as much as 200 cc. of sedimented material per liter of treated pulp within the first minute after treatment.

When the material is treated, of course, it should be permitted to remain in the settling tank for a unit of time sufficient to produce a substantial settling of the intermixed fine particles, after which the settled material is recovered from the tank and may thereafter be subjected to a suitable process of selective separation, to separate the valuable phosphate material from the impurities.

A suitable apparatus in which to carry out my

process is a settling or sedimentation tank, such as, for example, a thickener or hydroseparator as manufactured by the Dorr Company of New York city. In such an apparatus the settling zone is preferably an extensive and relatively shallow one, that is, a wide and thin layer of water. Thus in one installation, which is described by way of example only, the settling tank is a circular one, about 100 feet in diameter. The suspension of fine ore (which is a slurry collected from preceding parts of the plant) is pumped to the tank through a pipe or flume discharging in a downward direction at the center of the tank. From that point the pulp flows radially outward in all directions, in the form of a thin sheet, fifty feet in radius. The overflow around the circumferential lip or edge of the tank is a matter of inches or less in depth, depending upon the rate of pumping and flow of water, being in general of the order of about an inch or less in depth. Below the lip, the tank is cylindrical for a distance of about four feet and then has a bottom in the general form of a very flat inverted cone. The settled material collects on the bottom and is raked mechanically toward the discharge pipe at the apex of the cone. Thus the settling zone is about an inch, or less, in depth at the periphery, with a radius of fifty feet; and the particles need only settle through the depth of that zone, in order to fall below the lip of the tank, during the time required for the pulp to pass from the center to the rim of the tank. That time varies, of course, with different conditions, and is somewhat difficult to determine precisely. Calculation indicates an average time, for this particular illustrative installation, of around half a minute under certain conditions; less than two minutes in other cases, and a minute or less in still others, all depending on the rate of flow, the particular path of any given particle, and other factors. Once the particle settles sufficiently below the level of the rim of the tank so that it is not carried over by the overflowing water, it is caught, and can then settle at the bottom and be removed with the settled product. The sedimentation-acceleration reagents are preferably added in the feed to the tank, as in a mixing tank ahead of the feed pipe; although they can be added to the tank itself at the point where the inflow occurs.

Many other forms of apparatus and installation are suitable for application of my invention; but the foregoing is described simply as an example of one suitable form of apparatus.

It will be seen that my invention, at least according to one of its features, and when applied to a process for increasing the useful recovery of valuable phosphate fines by a commercial phosphate washer and concentrating plant, wherein phosphate ore, specifically Florida pebble phosphate, is mined, without grinding, in a manner producing a mixture including both coarse and finely divided particles of both valuable phosphate material and undesired impurities, such finely divided particles of both phosphate and impurities including many particles which are too fine to settle rapidly in water, provides an important improvement which constitutes a true process, in which the successive steps include first forming a pulp or aqueous suspension of such intermixed fine materials, then feeding the suspension to a settling tank, then treating the suspension (either in the tank or by addition to the feed) with a settling-acceleration reagent of the class described, which, in the case of certain ores may, under favorable conditions,

sometimes be caustic soda alone, but in other cases is one or more of the other reagents illustrated above, to increase the rate of settling of the intermixed fine particles of both phosphate materials and impurities after such treatment. The treated material is allowed to remain in the settling tank for a unit of time sufficient to produce a substantial settling of the intermixed fine particles so treated, after which the settled material may be removed from the tank and recovered for subsequent subjection to concentration treatment, to separate the valuable phosphate material from the impurities.

Another somewhat more specific embodiment of my invention is in a process for increasing the useful recovery of valuable phosphates by a commercial phosphate washer and concentration plant, usually operating on Florida rock, wherein the ore containing the phosphate rock is hydraulically mined and the resulting slurry is then fed to a settling tank, with or without intermediate treatment such as screening and the like, and in which the slurry comprises pieces of phosphate rock (i. e., phosphate mineral) of widely varying size, intermixed with impurities such as silica, sand and clay, but the material is of unconsolidated nature, so that it does not require any preliminary crushing or grinding, which is employed upon certain Russian phosphate ores. In this respect, the improvement may comprise the steps of treating the slurry, as fed to the settling tank, and preferably while it is free from any added froth flotation reagent (which might interfere with my treatment), with a settling-acceleration reagent of the class described. A suitable example is an alkaline reagent comprising an alkaline sodium silicate in an amount, and having an approximate composition, equivalent to about one pound of caustic soda, and about two pounds of sodium silicate, per ton of dry solids in the feed pulp. This treatment is found substantially to increase the rate of settling and to increase the amount of solids settled out per unit of time of settling operation. Thus more phosphate bearing material in the form of settled sediment is made usefully available for further treatment, such as subsequent steps of concentration of the phosphate. The final result is to give a higher yield of phosphate concentrates, and consequently a higher recovery of phosphate from the ore.

In a somewhat broader aspect, my invention is embodied in a similar process for increasing the useful recovery of valuable phosphate fines from a commercial phosphate mining and treating plant, wherein the phosphate ore is mined (hydraulically or by dry mining) in a manner which produces a mixture including both coarse and finely divided particles of both valuable phosphate material and undesired impurities such as silica, sand or clay, many of such finely divided particles, of both phosphate and impurities, being too fine to settle rapidly from an aqueous suspension. In this case, the improvement may be said to reside in first forming a suspension, in water, of such intermixed fine materials; then feeding the suspension to a settling tank; treating the suspension (either in the tank or before fed thereto) with one or more of the "settling-acceleration" reagents defined above, and in an amount and concentration sufficient to produce rapid sedimentation throughout the initial settling period, as during the first minute, and, preferably, to more than double the volume of settled material, as compared with material or

pulp not so treated, at all times throughout an initial settling period, as throughout the first three minutes of settling time. Such increase in the rate of settling is, in general, of the intermixed fine particles of both phosphate materials and impurities, as compared with their untreated settling rate. The thus-treated material or pulp is then allowed to remain in the settling tank for a unit of time sufficient to produce substantial settling of the intermixed fine particles. The settled material may, of course, be then recovered or removed, and thereafter subjected to concentration treatment, to separate the valuable phosphate material from the impurities.

Treatments of phosphate ore such as are involved in the hydraulic mining, washing or soaking procedures described as preceding the settling or sedimentation treatment of the present invention, are in general such as to necessitate the production of a pulp or slurry which is free of large size material (e. g., pieces plus about 14 mesh) and which has a content of solid material (comprising phosphate ore, i. e., phosphate mineral and impurities) of less than 40 per cent by weight, of the pulp—indeed more usually less than 30% and very often of the order of 10 to 15%, i. e., not more than 20%. The solid material is so suspended that rapid, economical natural settling of it is impossible. Thus, in pulps of the sort tested in the foregoing examples, less than about 40% of the solid material settles (without my treatment) in one minute of settling time, or usually, even in two minutes or more. For concentration and recovery of phosphate values from solid material such as is contained in such pulps, it is ordinarily prerequisite, for efficiency and economy, either that the material be dry or nearly dry, or at least that it be in a relatively thick pulp; for instance, practical wet concentration with reagents (e. g., tabling or froth flotation) of ore exemplified by the types containing Florida phosphate rock or debris, has been found to require, usually, a pulp feed of more than 50% solids content and preferably in most cases at least about 60%, and processes such as electrostatic concentration ordinarily require a dry feed of solid material. The great practical value of my process should therefore be manifest, particularly in achieving the recovery from pulps or slurries of an unavoidably dilute character, of a great deal more phosphate ore material (for subsequent concentration or other treatment) than it has heretofore been commercially practical to obtain.

The processes and reagents herein described, and the particular illustrative examples given, are the best embodiments of my present invention now known to me; but it is to be understood that the invention is not necessarily or specifically limited thereto, but may, under proper conditions, be carried out in other ways, without departure from its spirit, and within the scope of the following claims.

I claim:

1. In a process for improving the recovery of phosphate ore material for subsequent concen-

tration of phosphate values therefrom that is in the form of an aqueous pulp comprising a suspension of intermixed phosphate mineral and impurities in divided form as a result of hydraulically mining phosphate ore rock and screening out the large pieces of phosphate rock, said pulp having a content of said phosphate minerals and impurities of less than forty per cent, and the said suspension of said phosphate minerals and impurities being such that the major part of said phosphate mineral and impurities is not recoverable by natural settling within the first two minutes of settling time, the steps of feeding the pulp to a settling tank immediately after screening out the large pieces of phosphate rock and not later than the time the pulp is received in the settling tank accelerating the settling of phosphate mineral and impurities by producing and maintaining the pulp in an alkaline condition and adding a deflocculating or dispersing agent thereto, to more than double the volume of settled material, as compared with material not so treated, at the end of one minute of settling time following the time at which the pulp is allowed to commence settling, allowing said treated pulp to remain in the settling tank for a relatively short period of time sufficient to provide substantially accelerated settling of phosphate mineral and impurities within not more than substantially ten minutes immediately following the time the pulp is received in the settling tank, to thus provide a settled product which upon withdrawal from the tank represents a substantially increased recovery of the intermixed phosphate mineral and impurities as compared with settling of untreated material in substantially the same time, collecting the settled product from the settling tank and then for the first time subjecting the same to concentration treatment for recovery of phosphate values therefrom.

2. A process according to claim 1 in which the added agent comprises an alkaline sodium silicate in an amount, and having an approximate composition, equivalent to at least one pound of caustic soda and about one and one-half pounds of sodium silicate per ton of dry solids in the pulp.

3. A process according to claim 1 in which the added agent comprises sodium silicate.

4. A process according to claim 1 in which the added agent comprises wood pulp waste liquor materials.

5. A process according to claim 1 in which the added agent comprises material of the class consisting of alkaline sodium phosphate and molecularly dehydrated alkali phosphates.

6. A process according to claim 1 wherein the concentration treatment of the resultant settled product is by wet methods of concentration to obtain a wet phosphate product having increased content of useful phosphate material.

7. A process according to claim 1 wherein the concentration of the settled product is by flotation in order to produce an increased recovery of phosphate values.

DONALD S. PHELPS.

CERTIFICATE OF CORRECTION.

Patent No. 2,381,514.

August 7, 1945.

DONALD S. PHELPS.

It is hereby certified that error appears in the printed specification of the above numbered patent requiring correction as follows: Page 4, second column, line 34, for "re-pulsing" read --re-pulping--; page 8, second column, line 21, claim 1, strike out the period after "to" first occurrence and insert instead a comma; and that the said Letters Patent should be read with this correction therein that the same may conform to the record of the case in the Patent Office.

Signed and sealed this 25th day of December, A. D. 1945.

Leslie Frazer

(Seal)

First Assistant Commissioner of Patents.